

7 from 9 2-11

June 23, 1931.

E. ELGERUS

1,811,783

METHOD FOR MAKING WHITE AND BLEACHED WOOD PULP SUITABLE FOR  
THE MANUFACTURE OF PAPER WITHOUT ADDITION OF CELLULOSE

Filed March 28, 1929



Fig. 1



Fig. 2

Ernest Elgerus, Inventor,  
By *J. B. Townsend & Brickerstein*,  
Attorneys.

## UNITED STATES PATENT OFFICE

ERNST ELGÉRUS, OF NIKLASDORF-ON-THE-MUR, AUSTRIA

## METHOD FOR MAKING WHITE AND BLEACHED WOOD PULP SUITABLE FOR THE MANUFACTURE OF PAPER WITHOUT ADDITION OF CELLULOSE

Application filed March 28, 1929, Serial No. 350,778, and in Germany September 26, 1927.

This invention relates to a method for making white and bleached wood pulp suitable for the manufacture of paper without addition of cellulose.

5 Quite a number of methods have been proposed for utilizing the waste sulfite liquor, coming from the boilers in the manufacture of sulfite pulp. According to one of these methods the waste sulfite liquor is used for 10 treating disintegrated wood in a pressure boiler, into which steam of five atmospheres pressure is introduced, thus boiling the wood in the waste sulfite liquor at a temperature of about 128° C. After a treatment of about 15 3 to 4 hours the decomposed wood is separated into fibres in an edge mill: the disintegrated material may directly be used for the manufacture of wrapping paper and the like.

According to the invention the hot waste 20 sulfite liquor coming from the boilers in the manufacture of sulfite pulp is utilized in a more economical manner than that described above for decomposing wood for the manufacture of wood pulp, which can be used for making paper without addition of cellulose. I 25 have namely found, that excellent results in decomposing wood with waste sulfite liquor for the purpose described are also obtained, when the hot waste sulfite liquor is acting 30 upon wood without any further supply of heat such as introducing steam into the pressure vessel containing the wood to be treated and the waste sulfite liquor. It has been found that, in order to utilize completely the heat 35 content of the hot waste liquor so that the residual SO<sub>2</sub> content will exert the desired disintegrating and bleaching effect on the wood, it is only necessary to produce a certain pressure in the vessel, for example 3 atmospheres 40 or more. This can be effected, for instance, by pumping into the vessel so much of the hot waste liquor that the desired pressure is attained, and thereafter leaving the wood, without any further supply of heat to the 45 action of the hot liquor under the pressure thus attained for several hours for example three hours, or the desired amount of the hot waste liquor may be pumped into the treating vessel charged with wood and air or other 50 suitable gas pumped in with a compressor un-

til the desired pressure is attained, the wood being then left to the action of the liquor for the necessary length of time without any further supply of heat. The decomposition of the wood treated in this way is in about three 55 hours carried so far, that it can be disintegrated in an edge mill to slightly yellowish wood pulp suitable for making paper without addition of cellulose. If the time of treating the wood in the described manner is increased or the pressure during treatment 60 raised to pressures above three atmospheres the decomposition of the wood is carried so far, that nearly white wood pulp with good 65 mechanical properties is obtained.

The described process makes possible the full utilization of the heat- and SO<sub>2</sub>- content of the waste liquor for the production of a product, which on mechanical disintegration 70 gives a long-fibered white ground pulp, from which a printing paper may be made on a paper machine running at 150 meters speed without the addition of cellulose. The power consumption for the grinding of the wood treated by the present process is only 75 about one-half that used in the usual grinding process.

The annexed drawings show by way of example and schematically two small plants for carrying out the invention.

According to the scheme in Fig. 1 of the drawings the hot waste sulfite liquor in the sulfite boiler 3 is drawn off by a pump 4, when the sulfite boiling is finished and pumped into the pressure vessel 1, which has previously been filled with wood on a carriage 2. The pumping of hot waste sulfite liquor into the pressure vessel 1, is continued until a suitable superatmospheric pressure such as three atmospheres is obtained in the pressure 85 vessel 1. Then the wood is allowed to stand without further supply of heat under superatmospheric pressure in the waste sulfite liquor for several, say four hours. If necessary compressed air may be pressed into the 90 pressure vessel 1 during the treatment. When the treatment is finished the waste sulfite liquor is drawn off, the decomposed wood removed from the pressure vessel and disintegrated to pulp in an edge mill or the like.

The scheme shown in Fig. 2 of the drawings differs from the above scheme only by the fact, that the pressure vessel 1 is vertical instead of horizontal.

5 Instead of wood one can also treat in the same manner the chippings obtained by the decortication of wooden stems.

I claim:

1. A method for making bleached wood pulp which consists in treating wood for several hours at superatmospheric pressure with hot waste sulfite liquor without supplying any heat other than that contained in the liquor and disintegrating the treated wood 15 to mechanical wood pulp.

2. A method for making bleached wood pulp which consists in pumping hot waste sulfite liquor into a closed vessel filled with wood until superatmospheric pressure is obtained in the vessel, keeping the superatmospheric pressure in the vessel for several hours without supplying any heat other than that contained in the liquor and releasing the pressure in the vessel, removing the wood 25 from the vessel and disintegrating the treated wood to mechanical wood pulp.

3. A method for making bleached wood pulp which consists in pumping hot waste sulfite liquor into a closed vessel filled with wood until superatmospheric pressure of at 30 least three atmospheres is obtained in the vessel, keeping the superatmospheric pressure in the vessel for several hours without supplying any heat other than that contained in the liquor and releasing the pressure in the vessel, removing the wood from the vessel and disintegrating the treated wood to mechanical wood pulp.

4. A method for making bleached wood pulp which consists in pumping hot waste sulfite liquor into a closed vessel filled with wood, introducing compressed air into the vessel until superatmospheric pressure is obtained in the vessel, keeping the superatmospheric pressure in the vessel for several hours without supplying any heat other than that contained in the liquor and releasing the pressure in the vessel, removing the wood from the vessel and disintegrating the treated wood to mechanical wood pulp.

In testimony whereof I affix my signature.

ERNST ELGÉRUS.